

# UNITED STATES PATENT OFFICE.

HARRY S. MORK, OF BROOKLINE, AND GUSTAVUS J. ESSELEN, JR., OF SWAMPSOFT,  
MASSACHUSETTS, ASSIGNEES TO ARTHUR D. LITTLE, INC., OF CAMBRIDGE,  
MASSACHUSETTS, A CORPORATION OF MASSACHUSETTS.

## PROCESS OF MAKING COMBUSTIBLE MATERIAL.

1,416,493.

Specification of Letters Patent. Patented May 16, 1922.

No Drawing.

Application filed September 10, 1919. Serial No. 322,954.

To all whom it may concern:

Be it known that we, HARRY S. MORK, a citizen of the United States, and a resident of Brookline, in the county of Norfolk and State of Massachusetts, and GUSTAVUS J. ESSELEN, Jr., a citizen of the United States, and a resident of Swampscott, county of Essex, and State of Massachusetts, have invented a certain new and useful Process of 10 Making Combustible Material, of which the following is a specification.

Our invention relates to a combustible material composed mainly of alcohol, and particularly to such a material which may be made up into a solid mass which may be burned in the open, or in a suitable container.

The objects of our invention are to produce such a permanent material which is inexpensive to manufacture, which will burn freely without liquefaction, which will not sweat or exude liquid to an objectionable degree, which will not form a crust on the surface when the flame is extinguished, which will quickly cool when the flame is extinguished, which may be readily relighted, and which will leave practically no residue.

A further object of the invention is the production of a combustible material, the 30 luminosity of the flame produced on combustion of which may be modified by proper selection of the materials employed, the character of the flame being luminous or non-luminous, according to such selection.

35 A further object of the invention is to provide a process or method of making a combustible material as above described, in which the loss of material by evaporation or otherwise will be negligible, which is not limited to the use of any particular grade of the solid material employed, and in which a portion, at least, of the material used in the process and which may be undesirable or objectionable in the combustible material 40 of the invention may be removed and conserved.

These and further objects will more fully appear in the following specification and claims.

50 In producing the product of the invention a suitable cellulose nitrate is dissolved in a volatile combustible solvent or solvent mixture. The solution is coagulated in a more or less comminuted or granular jellied con-

dition, as distinguished from a single coherent mass, by means of an excess of a non-solvent liquid. The excess liquid is removed from the comminuted granules, which are then ready for the next step in the process.

A second solution of cellulose nitrate is prepared, to which is added a liquid non-solvent, in quantity sufficient to bring the solution almost, but not quite, to the point of coagulation. Into this second solution the jelly granules, or lumps, are introduced, and if the proportions of granules and the second solution are properly regulated the mixture will set to a solid mass without appreciable exudation of liquid.

The last mentioned step of the process 70 may be carried out in the container in which the material is to be marketed and burned, or said final mixture may be made in any suitable vessel and the product cut or otherwise shaped to any form desired.

75 The cause of the setting, when the granules are mixed with the solution of the second step of the process, is believed to be due to diffusion of the non-solvent from the jelly granules or lumps into the solution of the second step to a degree which causes coagulation of the solution, and binding of the entire mixture into a solid mass.

80 The product made by the process herein described is a permanent jell having a minimum tendency to exude liquid on standing. The tendency of the jellied granules is toward expansion, the tendency of the solution which is mixed with the granules is toward contraction, but as the proportion of granules is largely in excess of that of the solution, the expansive effect exceeds the contractive effect, and the tendency of the solidified product as a whole is therefore toward expansion, and there will be no exudation 90 of liquid.

85 As an illustration of one method of carrying out the process, approximately 5 grams of cellulose nitrate are dissolved in about 20 cc. of ethyl acetate and 70 cc. of denatured alcohol. This solution is mixed with 100 80 cc. of denatured alcohol with vigorous agitation, whereby the solution is coagulated in the form of gelatinous lumps or granules suspended in a relatively large 105 amount of liquid. The granules are allowed to soak in this liquid to permit a part, at least, of the solvent to diffuse from the gran-

ules into the liquid, to add to the firmness of the granules. This soaking may take from one-half to one hour, but longer soaking will not be harmful. After the soaking operation has been carried as far as desired the excess liquid is drained from the granules.

A second solution is now made by dissolving approximately 1.5 grams of cellulose nitrate in about 13 cc. of a mixture of equal parts of ethyl acetate and denatured alcohol. After solution is complete about 32 cc. of denatured alcohol are added with stirring. If a suitable cellulose nitrate be employed no coagulation will take place and the mixture will be fluid.

The second mixture is added to the granules produced in the first stage, in amount sufficient to cover the granules, and allowed to stand until the entire mass solidifies. The product may now be packed and is ready for use.

All of the steps of the process may be carried out at room temperature.

The general operation of the process, and a concrete example thereof, have been described, but it is to be understood that the invention is not limited to the specific ingredients and the exact proportions given. Any solvent or mixture of solvents of suitable combustibility may be employed in the preparation of the granules or lumps, or in the liquid or liquids of the second step of the process. The solvents employed are solvents of cellulose nitrate of widely differing grades, and the process and compound are not confined to the use of cellulose nitrate of any particular degree of nitration.

The first mixture need not be made up in the form of lumps or granules. The nitro-cellulose solution may be forced through small orifices into the non-solvent, as in the manufacture of artificial silk, thereby forming the gelatinous granules in filamentary form, and the filamentous particles may be formed into a solid mass as before.

The mixture of the gelatinous granules and the liquid of the second step may be made in the containers in which the product is to be vended and burned; the mixture may be made in a separate vessel and poured into the container before it jells; or the mixtures may be united in a large receptacle and, after solidification of the final mixture, be cut or otherwise formed to any required size and shape and packed as desired.

By proper selection of the combustible liquids absorbed in the cellulose nitrate, the luminosity of the flame produced on combustion of the product may be modified. A product, to be employed for heating purposes only, may produce a non-luminous, or feebly luminous flame. One burning with a luminous flame, and which may be used for heating and illuminating purposes, may be produced.

For illuminating purposes the mixture may be made by the addition of from 10% to 20% of benzol, gasoline or other coal-tar or petroleum hydrocarbon, figured on the total solvent employed.

If desired the product may be colored by the addition of any suitable coloring matter, and the odor may be modified, or masked, by the addition of small quantities of odoriferous substances.

By the use of suitable proportions of denatured alcohol and methyl or wood alcohol in the solutions and coagulating liquid, a fuel which will burn with non-luminous flame may be produced.

As examples of solvents other than ethyl acetate, may be mentioned ether-alcohol mixtures, methyl acetate, mixtures consisting chiefly of ethyl alcohol, acetone, other ketones, etc.

By draining the excess liquid from the granules and successively supplying fresh quantities of non-solvent, the percentage of solvent in the granules will be gradually reduced and may be recovered from the drained off liquid by known means.

For commercial and manufacturing reasons the preferred cellulose nitrate for use in the process is that usually referred to as pyroxylin. This material, has a nitrogen content between 10.5% and 12.6%. It is completely soluble in butyl acetate with a viscosity of 45-50. In measuring the viscosity, a 5% solution of the pyroxylin in butyl acetate is used in an Ostwald viscometer at a temperature of 25° C., the viscosity being expressed in relation to that of glycerine taken at 100.

The above pyroxylin is given as an example only, and applicants desire to have it understood that any other cellulose nitrates having a nitrogen content which is soluble in the solvents indicated, may be employed in the process.

In accordance with the provisions of the patent statutes the principle of the invention has been described, together with what is now considered to be the best embodiment thereof; but it is to be understood that the embodiment described is merely illustrative and that the invention may be carried out in other ways.

Having now described the invention what is claimed and desired to be secured by Letters Patent, is:—

1. The process of making an infusible solidified combustible material, which comprises dissolving in a volatile combustible compound the formula of which contains a carbonyl group, a cellulose nitrate having a nitrogen content which renders it soluble in the compound, coagulating the solution in an excess of a volatile combustible non-solvent, and removing the excess of the non-solvent.
2. The process of making an infusible

solidified liquid combustible material, which comprises dissolving pyroxylin in a volatile combustible solvent the formula of which contains a carbonyl group, coagulating the 5 solution in a volatile combustible non-solvent; preparing a second solution of pyroxylin in a suitable solvent, said second solution being close to the point of coagulation; and mixing the coagulated solution with the 10 non-coagulated solution to solidify the mixture.

3. The process of making an infusible solidified liquid combustible material, which comprises dissolving pyroxylin in a volatile 15 combustible solvent the formula of which contains a carbonyl group, coagulating the solution in an excess of a volatile combustible non-solvent, removing the excess of non-solvent, preparing a second solution of 20 pyroxylin close to the point of coagulation in a suitable solvent, and mixing the coagulated solution with the non-coagulated solution to solidify the mixture.

4. The process of making an infusible 25 solidified liquid combustible material, which comprises dissolving pyroxylin in a combustible solvent the formula of which contains a carbonyl group, and coagulating the solution into disjoined masses by the means of 30 an excess of a volatile combustible non-solvent, and removing the excess.

5. The process of making an infusible solidified liquid combustible material, which comprises dissolving pyroxylin in a volatile 35 combustible solvent the formula of which contains a carbonyl group and alcohol, coagulating the solution into disjoined masses by means of an excess of alcohol, and removing the excess of the alcohol.

40 6. The process of making an infusible solidified liquid combustible material, which comprises dissolving pyroxylin in ethyl acetate, adding a non-solvent in quantity sufficient to coagulate the solution in the 45 form of disjoined masses, preparing a second solution by dissolving pyroxylin close to the point of coagulation in ethyl acetate, and mixing the disjoined masses with the second solution to solidify the mixture.

50 7. The process of making an infusible solidified liquid combustible material, which comprises dissolving pyroxylin in ethyl acetate, adding alcohol in quantity sufficient to coagulate the solution in the form of 55 disjoined masses, preparing a second solution by dissolving pyroxylin close to the point of coagulation in ethyl acetate and alcohol, and mixing the disjoined masses with the second solution to solidify the mixture.

60 8. The process of making an infusible

solidified liquid combustible material, which comprises dissolving pyroxylin in ethyl acetate, adding an excess of alcohol in quantity sufficient to coagulate the solution in the form of disjoined masses, removing the excess, 65 preparing a second solution by dissolving pyroxylin close to the point of coagulation in ethyl acetate and alcohol, and mixing the disjoined masses with the second solution to solidify the mixture. 70

9. The process of making an infusible solidified liquid combustible material, which comprises dissolving 5 grams of cellulose nitrate in approximately 20 cc. of ethyl acetate and 70 cc. of denatured alcohol, adding to 75 approximately 80 cc. of denatured alcohol with vigorous agitation, whereby the mixture is coagulated in the form of disjoined masses in an excess of liquid, allowing the masses to soak in the liquid; making a coagulating solution by dissolving 1.5 grams of cellulose nitrate in approximately 6.5 cc. of ethyl acetate and approximately 6.5 cc. of denatured alcohol, adding to the said coagulating solution approximately 32 cc. of denatured alcohol with agitation, and mixing the coagulating solution with the disjoined masses, whereby a solid mixture is produced. 80

10. The process of making an infusible solidified liquid combustible material, which comprises dissolving 5 grams of pyroxylin in approximately 20 cc. of ethyl acetate and 70 cc. of denatured alcohol, adding approximately 80 cc. of denatured alcohol with vigorous agitation, whereby the mixture is 95 coagulated in the form of disjoined masses in an excess of liquid, allowing the masses to soak in the liquid; making a coagulating solution by dissolving 1.5 grams of pyroxylin in approximately 6.5 cc. of ethyl acetate and 100 approximately 6.5 cc. of denatured alcohol, adding to the said coagulating solution approximately 32 cc. of denatured alcohol with agitation, adding a hydrocarbon distillate, 105 and mixing the coagulating solution with the disjoined masses, whereby a solid mixture is produced.

This specification signed and witnessed this 20th day of August, 1919.

HARRY S. MORK.  
GUSTAVUS J. ESSELEN, JR.

Witnesses to the signature of Harry S Mork:

LAWRENCE HEMENWAY,  
CARL C. SORENSEN.

Witnesses to the signature of Gustavus J Esselen, Jr.:

EARL P. STEVENSON,  
CLARENCE J. WEST.